

## UNITED STATES PATENT OFFICE

2,290,719

## TYPOGRAPHICAL PLATE

Jeptha H. Todd, Kansas City, Mo.

No Drawing. Application June 5, 1941,  
Serial No. 396,777

3 Claims. (Cl. 101—395)

This invention relates to improvements in typographical or printing plates and refers more particularly to printing plates produced from an improved plastic composition which has satisfactory structural strength, a proper affinity for ink, and which will withstand heat necessary to transfer typographical forms, cuts and half-tones from matrices and will accept and reproduce exceedingly fine detail.

Heretofore, attempts have been made to produce printing plates of plastic material. As early as 1892, the use of vulcanized clay, shellac and wood pulp was suggested by Steele in Patent No. 486,572. In 1901, stereotypes of Celluloid were produced according to the invention of the Danish patentee, Madsen, as described in Patent No. 672,534. Novotny, in 1921, advocated the use of Bakelite, in Patent No. 1,377,516. Reinforced acetyl cellulose was recommended by Richter in 1931, according to Patent No. 1,794,322. A cellulosic plastic, combined with a metal compound such as lead carbonate and iron oxide was described by Boutwell in Patent No. 2,219,587, issued in 1940.

All of these attempted improvements, in so far as the printing industry is concerned, were of doubtful success. For one reason or another, the typographical forms or plates did not meet the requirements of the printer. Hardness and structural strength, with a certain amount of flexibility, are necessary, as well as the ability of the composition to receive and reproduce the fine details of half-tone plates and stereotypes. The affinity of the composition for ink has been another difficulty that was not overcome in some instances.

The process of the present invention comprises a series of steps in the production of a printing plate, that has been found to meet the requirements of the trade. The steps of the process will be described in connection with the reproduction of a copper plate or half-tone, or zinc etching, as the detail is more minute and therefore more difficult to reproduce. It must be understood, however, that any type of printing composition or printing characters may be transferred to a printing plate in a similar manner.

The process for compounding the plastic dough from which the plastic printing plate is made is by use of a powerful rolling machine constructed on a heavy base with two parallel rollers 30 inches in length and 12 inches in diameter, rolling in opposite directions which causes a kneading action when material is placed between them. One roller is heated to 200° F.

10 and the other is cooled with circulating water. A mixture of 2 pounds 5 ounces shellac, 1 pound 14 ounces wool flock, 12 pounds basic lead sulphate and a small quantity of black dye to add color is mixed thoroughly and run between the rollers. The moisture in the shellac and high pressure forces the powder into the shellac and the mixture becomes moist and kneads itself in the revolving machine. After being thoroughly mixed, it is removed from the hot roller in the form of a slab about  $\frac{1}{8}$  inch in thickness, 26 inches wide and 36 inches long. When removed, it is placed on a flat surface and within a few minutes is in a hardened plastic state. It is from this material that the plastic printing plate is made.

15 In order to make a negative plastic printing plate, it is necessary to mould this by using a positive matrix. This matrix is made from the original half-tone or set-up type or printing characters by placing same with the printing face over uncured Bakelite matrix material, which is in general use for the same type of construction in rubber printing plates. With 20 heat and pressure, the plate to be reproduced is pressed into Bakelite and cured at 300° F. for a period of 15 minutes and when removed from the press the plate is removed from the Bakelite leaving a hard cured indented matrix carrying the exact positive impression of the negative plate.

25 From the plastic dough previously mentioned a piece is cut to the size of the piece to be reproduced. It is placed on a steam-heated table of 200° F. and allowed to soften. It is then placed over the indented matrix and together the matrix and plastic plate are placed in a hydraulic press and the press is closed under pressure of from 25 to 100 tons, depending upon the size of the plate being reproduced. When the press is closed so that the plastic dough is thoroughly pressed into the intaglio mould and of the proper thickness, the closing process is discontinued but the pressure is held. Through a cooling process of circulating refrigerated water through the top and bottom platens of the hydraulic press, the plastic is cooled and when removed from the press is easily separated from the matrix leaving a negative perfect reproduction of the matrix. Through 30 the action of intense pressure while in a warm and flexible state and the cooling process, the plastic plate assumes a hardness greater than lead, zinc or a nickel stereotype, but will route and tool as metal.

35 The time required for reproduction of a plastic

printing plate from the original metal half-tone or electrotype is approximately 2 minutes to complete the matrix and 10 minutes to make the first plastic plate. However after this is accomplished, additional plastic printing plates can be produced identical with the first at the rate of one for each 5-minute period and it has been demonstrated that as many as 20 or more identical plates may be produced from the matrix.

After the negative impression is taken from the Bakelite matrix, it is sawed to size and mounted and planed to type-high or to a proper thickness for incorporating into the conventional type of printing bases in general use. Composition typographical forms or plates of this material can be drilled for tacking to a base or can be glued to a base, depending upon the manner in which the printer intends to use the plate for reproduction purposes. The composition has a very high affinity for ink and will withstand considerably more use and abuse than the average printing plate in general use.

In place of the wool flock suggested as a constituent of the mix above, cotton, rayon or other types of fibre flock which have a sufficient degree of fineness and strength may be used. Instead of lead sulphate, lithopone, consisting chiefly of a mixture of zinc sulphide and barium sulphate, has been used with satisfaction. On occasions, a small amount of ethyl cellulose has been found to give the plastic added toughness, but care must be taken to restrict the amount to avoid any likelihood of ignition. Particularly during the mixing process and from the heat of the press when the impression is made from the positive matrix, care must be taken to avoid excess temperatures. In the example of a typical mix described heretofore, from 2 to 4 ounces of ethyl cellulose to 2 pounds 5 ounces of shellac, 1 pound 14 ounces of wool flock and 12 pounds of lead sulphate proved satisfactory.

Plates made according to this method have been used for the reproduction of half-tones and zinc etchings for 20,000 or more reproductions with little or no indication of wear. Typographical forms or plates made according to the method afford a rugged construction, able to withstand

pressures and wear from operations in the press, plates which are not easily defaced due to handling and storage and plates which give a perfect reproduction of fine lines and images from copper plates and zinc etchings.

In addition to the fine reproductions obtained by using this plastic printing plate, it affords the printer a great saving in both time and money. In case the printer desires to complete 10 a large run and is required to mount several copies on his press so that they may all be printed in one operation, it is possible to obtain these cuts at the rate of speed previously mentioned and at a great saving over metal cuts previously used.

The general custom followed by a printer is that he does not use the original cut supplied from a photograph or artist's drawing but uses 20 electrotypes reproduced from the original. The plastic printing plate affords this reproduction at a saving of time and expense.

It will be understood that certain features and sub-combinations are of utility and may be employed without reference to other features and 25 sub-combinations. This is contemplated by and is within the scope of my claims. It is further obvious that various changes may be made in details within the scope of my claims without departing from the spirit of my invention. It is, 30 therefore, to be understood that my invention is not to be limited to the specific details shown and described.

Having thus described my invention, I claim:

1. A printing plate composed of a mixture of 35 a binder, a fibre flock and a filler selected from the group of materials consisting of basic lead sulfate and lithopone.

2. A printing plate composed of a mixture of shellac, a fibre flock and a filler selected from 40 the group of materials consisting of basic lead sulfate and lithopone.

3. A printing plate composed of a mixture of 45 a binder, a fibre flock and a filler selected from the group consisting of basic lead sulfate and lithopone and a minor portion of ethyl cellulose.

JEPHTHA H. TODD.